

3,397,986

PHOTOGRAPHIC EMULSION STABILIZED WITH  
BIS(p-ACYLAМИDOPHENYL)DISULFIDES

Allan G. Millikan and Arthur H. Herz, Rochester, N.Y.,  
assignors to Eastman Kodak Company, Rochester, N.Y.,  
a corporation of New Jersey  
No Drawing. Filed Dec. 29, 1964, Ser. No. 421,994  
14 Claims. (Cl. 96—109)

## ABSTRACT OF THE DISCLOSURE

The stabilization against fog of photographic silver halide emulsions using bis(p-acylamidophenyl)disulfides is disclosed.

This invention relates to stabilized photographic compositions. More particularly, this invention relates to the stabilization of photographic silver halide emulsions. In a specific aspect, this invention relates to inhibiting development of spontaneous fog without adversely affecting the sensitivity of a photographic silver halide emulsion.

It is known that photographic silver halide emulsions on storage tend to lose sensitivity and to become spontaneously developable without exposure to light. There is normally a detectable amount of the silver salt reduced during development in the area where no exposure was given; this is commonly called "fog" and sometimes called "chemical fog" where it is necessary to distinguish between it and the effects of accidental exposure to radiation.

Certain organic disulfides have been described as being effective in preventing an increase in fog and to stabilize or control the keeping quality of photographic emulsions. However, many of these organic disulfides are not effective antifoggants unless they are used in combination with other materials and still others cause objectionable desensitization of the emulsion. For example, U.S. Patent 2,440,110 discloses that organic disulfides such as diphenyl disulfide or ditolyl disulfide must be used in combination with sulfinic or seleninic acids or their salts to obtain acceptable stabilization. It is evident, therefore, that the state of the art will be enhanced by providing photographic silver halide emulsions which are stabilized by organic disulfides which are not subject to the aforementioned deficiencies.

Accordingly, it is an object of this invention to provide stabilized photographic silver halide emulsions.

Another object of this invention is to provide a method for stabilizing photographic silver halide emulsions.

Another object of this invention is to provide a method of stabilizing photographic silver halide emulsions without adversely affecting, to any substantial extent, the sensitivity of the emulsion.

Still another object of this invention is to provide photographic silver halide emulsions which are stabilized with organic disulfides.

Other objects will become apparent from an examination and consideration of the specification and claims that follow.

In accordance with this invention, it has been found that photographic silver halide emulsions can be stabilized and the development of spontaneous fog substantially inhibited by the use of at least one bis(p-acylamidophenyl) disulfide having the formula:



where each R is a trifluoromethyl, alkyl or aryl radical.

In view of the teachings of U.S. Patent 2,440,110, it

could not have been predicted that the substituted phenyl disulfides employed in the practice of this invention would be effective stabilizers for photographic silver halide emulsions and prevent the development of spontaneous fog. Thus, U.S. Patent 2,440,110 indicates that structurally closely related organic disulfides, i.e., aryl disulfides having unsubstituted aromatic rings and aromatic rings containing such substituents as carboxylic acid, primary amino or alkyl groups, do not exhibit antifoggant activity. Furthermore, as shown by Example 4, set out hereinafter, other seemingly slight changes in the chemical structure of the disulfide have significant deleterious effects upon the speed, stability and/or development of spontaneous fog of photographic silver halide emulsions containing such disulfide.

As already indicated, the stabilizers employed in the practice of this invention have the formula:



where each R is a trifluoromethyl, alkyl or aryl radical. It is obvious that the



group is an acyl radical derived from an aliphatic or aromatic carboxylic acid. The R groups, except in the case of trifluoromethyl, are hydrocarbon and generally contain up to about 20, preferably up to 10, carbon atoms. The preferred alkyl groups contain 1-10 carbon atoms. Suitable R groups include, for example, trifluoromethyl, methyl, ethyl, propyl, isopropyl, n-butyl, isobutyl, octyl, decyl, dodecyl, eicosyl, phenyl, tolyl, naphthyl, anthryl, and the like. Hence, examples of the disulfide employed in the practice of this invention include

bis(p-acetamidophenyl)disulfide,  
bis(p-trifluoroacetamidophenyl)disulfide,  
bis(p-butylramidophenyl)disulfide,  
bis(p-propionamidophenyl)disulfide,  
bis(p-octanamidophenyl)-disulfide,  
bis(p-decanamidophenyl)disulfide,  
bis(p-pentadecanamidophenyl)disulfide,  
bis(p-benzamidophenyl)disulfide,  
bis(p-naphthamidophenyl)disulfide

and the like.

A convenient method for preparing the bis(p-acylamidophenyl)disulfide stabilizers employed in practicing this invention comprises reacting 4,4'-diamidodiphenyl disulfide with the appropriate carboxylic acid anhydride as represented by the following equation:



where each R is as defined hereinbefore. The reaction generally takes place at relatively mild temperatures, for example, temperatures up to about 100° C. Normal atmospheric pressures are preferably employed although pressures substantially below or above normal atmospheric pressures can be used. If desired, the reaction can be carried out in an inert organic vehicle, and will go to completion in a relatively short period, generally not more than about 4 hours. The resulting bis(p-acylamidophenyl)disulfides can then be isolated by conventional procedures, for example, filtering, washing and drying. The synthesis of bis(p-acetamidophenyl)disulfide by this procedure is shown in Berichte 38, p. 1134 (1905) and

Beilstein Organ. Chem., vol. XIII, p. 544 (1930). As is obvious to those skilled in the art, other bis(p-acylamido-phenyl)disulfides used in practicing this invention can be prepared in the same manner by employing the appropriate carboxylic acid derivative in the reaction.

The stabilizing concentration of the bis(p-acylamido-phenyl)disulfide employed in a given emulsion is subject to wide variation, depending upon the effects desired, degree of ripening, silver content of the emulsion, etc. In general, a concentration in the range of about .001 to about 10, preferably about .1 to about 1 gram per mole of silver halide is adequate. The stabilizer can be incorporated directly into the silver halide emulsion layer or it can be present in an adjacent layer. It is generally desirable to use higher concentrations of stabilizer when it is used in an adjacent layer rather than in the silver halide emulsion layer. Exposure of the treated emulsion in conventional photographic testing apparatus such as an intensity scale sensitometer, will reveal the most advantageous concentration for the present stabilizers in a particular emulsion. Such techniques are well known to those skilled in the art.

The stabilizers of this invention can be added to the photographic composition using any techniques suitable for this purpose. For example, they can be dissolved in a suitable solvent and added directly to the silver halide emulsion or they can be added to the emulsion in the form of a dispersion similar to the technique used to incorporate certain types of color forming compounds (couplers) in a photographic emulsion. The solvent should be selected so that it has no harmful effects upon the emulsion, in accordance with usual practice, and organic solvents or diluents are preferred. Examples of suitable solvents or diluents include ethanol, acetone or the like.

The stabilizing addenda employed in the practice of this invention can be used in various kinds of photographic emulsions. In addition to being useful in orthochromatic, panchromatic and infrared emulsions, they are also useful in X-ray and other non-optically sensitized emulsions. They can be added to the emulsions before or after any optically sensitizing dyes which may be used. They are particularly effective in sulfur and gold sensitized silver halide emulsions. Various silver salts can be used as sensitive salts, including, for example, silver bromide, silver iodide, silver chloride or mixed silver halides such as silver chlorobromide, silver bromoiodide or silver chloroiodide. The subject addenda can be used in emulsions intended for color photography, for example, emulsions containing color forming couplers or emulsions to be developed by salts containing couplers or other color generating materials.

In the preparation of the silver halide dispersions employed for preparing silver halide emulsions there can be employed as the dispersing agent for the silver halide in its preparation, gelatin or some other colloidal material such as colloidal albumin, a cellulose derivative or a synthetic resin, for example, a polyvinyl compound, although gelatin is preferred.

The photographic emulsions stabilized according to this invention can be coated on a wide variety of supports. Typical supports include those generally employed for photographic elements, as exemplified by cellulose nitrate film, cellulose acetate film, polyvinyl acetal film, polystyrene film, polyethylene terephthalate film and related films of resinous materials as well as glass, paper, metal, wood and the like. Supports such as paper that are coated with  $\alpha$ -olefin polymers, particularly polymers of  $\alpha$ -olefins containing 2-10 carbon atoms, as for example, polyethylene, polypropylene, ethylene butene copolymers and the like, can also be employed.

In addition to the antifogging addenda, the photographic emulsions and elements can also contain additional additives, particularly those known to be beneficial in photographic emulsions, as exemplified by opti-

cal sensitizers, speed increasing materials, gelatin hardeners, plasticizers and the like.

This invention can be further illustrated by the following examples of preferred embodiments thereof although it will be understood that these examples are included merely for purposes of illustration and are not intended to limit the scope of the invention unless otherwise specifically indicated.

#### Example 1

The disulfides disclosed herein stabilize photographic emulsions against increases in fog and decreases in speed even upon storage at increased temperatures and humidity. To illustrate, bis(p-acetamidophenyl)disulfide is incorporated into a negative, high speed gelatin silver bromoiodide emulsion containing a yellow dye forming coupler. The emulsion is coated on a cellulose acetate film base. For comparison, three samples of the identical emulsion, one sample containing no antifogging compound, one containing ditolyl disulfide and one containing diphenyl disulfide are coated on cellulose acetate film base in the same manner. Samples of the prepared photographic elements are then incubated for 7 days at 120° F. and 50% relative humidity, exposed for  $\frac{1}{25}$  second in the form of film strips in an intensity scale sensitometer (Kodak Type Ib) and developed for 12 minutes at 75° F. The developer employed has the following formula:

|    |                                                                                 |       |      |
|----|---------------------------------------------------------------------------------|-------|------|
| 30 | N-ethyl - $\beta$ - methanesulfonamidoethyl-3-methyl-4-<br>aminoaniline sulfate | ----- | 2.0  |
|    | Sodium sulfite (anhydrous)                                                      | ----- | .6   |
|    | Sodium carbonate (anhydrous)                                                    | ----- | 30.0 |
|    | Water to 1.0 liter.                                                             |       |      |

35 A negative silver image and a yellow dye image is formed. The silver image and the residual silver halide are removed by treatment with a conventional ferricyanide bleach followed by a hypo fixing bath leaving a yellow negative dye image.

40 The results of sensitometric tests on the samples are summarized by the data set out in Table 1 below. In Table 1, as well as in the tables appearing in the following examples, speeds indicated are a function of the exposure necessary to give a density of 0.2 above background fog, the initial control speed being taken as 100 in each case; and the concentrations of addenda, if any, are indicated as grams of addenda per mole of silver halide.

| 50 | Addenda                             | Concen-<br>tration of Adden-<br>da (grams/<br>mole of AgX) | After 7 days at 120° F.<br>50% relative humidity |     |
|----|-------------------------------------|------------------------------------------------------------|--------------------------------------------------|-----|
|    |                                     |                                                            | Speed                                            | Fog |
|    | Control                             | 0                                                          | 100                                              | .43 |
| 55 | Bis(p-acetamidophenyl)<br>disulfide | .25                                                        | 94                                               | .20 |
|    | Ditolyl disulfide                   | .185                                                       | 79                                               | .49 |
|    | Diphenyl disulfide                  | .164                                                       | 78                                               | .47 |

60 As can be observed from the above table, the bis(p-acylamidophenyl)disulfides of this invention impart substantial stabilizing and antifogging properties to photographic silver halide emulsions. It is also significant to note that the practice of this invention does not result in substantial loss in speed with the improved stability. In contrast, Table 1 illustrates that aryl disulfides having unsubstituted aromatic rings or aromatic rings containing such substituents as alkyl groups are ineffective to impart stabilizing or antifogging properties to photographic silver halide emulsions. As shown in U.S. Patent 2,440,110, such aryl disulfides require the presence of various sulfonic or seleninic acids or salts to exhibit any stabilizing effects. Such additional additives are, of course, not necessary with the specific organic disulfides employed in the practice of this invention.

## Example 2

A bis(p-acylamidophenyl)disulfide is added from a substantially neutral solution to a negative, high speed, orthochromatically sensitized gelatino silver bromoiodide emulsion containing a pyrazolone magenta dye forming coupler. A comparison sample is made with an identical batch of emulsion which contains no antifoggant compound. The coating, incubation, exposure, developing and processing procedures of Example 1 are repeated except that the exposure is for  $\frac{1}{50}$  second rather than  $\frac{1}{25}$  second. In 10 these runs test samples are also exposed in the sensitometer

5

deleterious affect on the stability and/or speed of the photographic silver halide emulsion. To illustrate, the procedure of Example 3 is repeated with bis(p-acetamidophenyl)disulfide and bis[o-(N-ethyl)acetamidophenyl] disulfide which has the formula:



The results of sensitometric tests are as follows:

TABLE 4

| Addenda                                   | Concentration of Addenda (grams/mole of AgX) | Initial Test |     | After 7 days at 120° F., 50% relative humidity |     | After 14 days at 120° F., 50% relative humidity |     |
|-------------------------------------------|----------------------------------------------|--------------|-----|------------------------------------------------|-----|-------------------------------------------------|-----|
|                                           |                                              | Speed        | Fog | Speed                                          | Fog | Speed                                           | Fog |
| Control                                   | 0                                            | 100          | .14 | 102                                            | .21 | 33                                              | .78 |
| Bis(p-acetamidophenyl)disulfide           | .09                                          | 110          | .09 | 120                                            | .10 | 78                                              | .18 |
| Do                                        | .30                                          | 95           | .10 | 112                                            | .10 | 73                                              | .18 |
| Bis[o-(N-ethyl)acetamidophenyl]-disulfide | .06                                          | 132          | .12 | 107                                            | .18 | 60                                              | .30 |
| Do                                        | .40                                          | 110          | .11 | 105                                            | .12 | 62                                              | .18 |

directly after coating. The results of sensitometric tests are as follows:

As will be observed from the above table, the bis[o-(N-ethyl)acetamidophenyl]disulfide, although quite closely

TABLE 2

| Addenda                         | Concen-<br>tration of Addenda<br>(grams/mole<br>of AgX) | Initial Test |     | After 7 days at<br>120° F., 50% rela-<br>tive humidity |     |
|---------------------------------|---------------------------------------------------------|--------------|-----|--------------------------------------------------------|-----|
|                                 |                                                         | Speed        | Fog | Speed                                                  | Fog |
| Control                         | 0                                                       | 100          | .25 | 87                                                     | .45 |
| Bis(p-acetamidophenyl)disulfide | .25                                                     | 83           | .19 | 95                                                     | .29 |

Similar results are obtained when bis(p-trifluoroacetamidophenyl)disulfide, bis(p-propionamidophenyl)disulfide or bis(p-butyramidophenyl)disulfide is substituted for 35 bis(p-acetamidophenyl)disulfide in the above procedure.

## Example 3

A typical bis(p-acylamidophenyl)disulfide, as described herein, is incorporated into a sulfur and gold sensitized negative, high-speed gelatino silver bromoiodide solution which is panchromatically sensitized with a cyanine dye. A comparison sample is made with an identical batch of emulsion which contains no antifoggant compound. These emulsions are coated on cellulose acetate film supports. 45 Samples of the prepared photographic elements, either directly after coating or after incubation for 7 days at 120° F. and 50% relative humidity, are exposed in the

related structurally to bis(p-acetamidophenyl)disulfide shows a substantial deleterious effect upon the speed and/or fog of a photographic emulsion when it is used in place of the latter. This same deleterious effect is exhibited by other ortho substituted aryl disulfides such as di-o-formylethylaminodiphenyldisulfide when they are employed in the above procedure.

Thus, this invention provides silver halide emulsions that are stabilized with antifoggant addenda which do not cause substantial desensitization or loss in speed.

Although the invention has been described in considerable detail with reference to certain preferred embodiments thereof, it will be understood that variations and modifications can be effected without departing from the spirit and scope of the invention as described hereinabove and as defined in the appended claims.

TABLE 3

| Addenda                         | Concen-<br>tration of Addenda<br>(grams/mole<br>of AgX) | Initial Test |     | After 7 days at<br>120° F., 50% rela-<br>tive humidity |     |
|---------------------------------|---------------------------------------------------------|--------------|-----|--------------------------------------------------------|-----|
|                                 |                                                         | Speed        | Fog | Speed                                                  | Fog |
| Control                         | 0                                                       | 100          | .14 | 102                                                    | .20 |
| Bis(p-acetamidophenyl)disulfide | .09                                                     | 110          | .09 | 120                                                    | .10 |
| Do                              | .3                                                      | 95           | .10 | 112                                                    | .10 |

form of film strips in an intensity scale sensitometer (Kodak Type Ib), developed for 5 minutes at 68° F. in 60 Kodak Developer DK-50 and fixed, washed and dried in the conventional manner. The results of sensitometric tests are listed above.

Similar results are obtained when bis(p-acylamidophenyl)disulfides such as bis(p-butyramidophenyl)disulfide, bis(p-naphthamidophenyl)disulfide, bis(p-octamidophenyl)disulfide or bis(p-pentadecanamidophenyl)disulfide are substituted for bis(p-acetamidophenyl)disulfide in the above procedure.

## Example 4

As pointed out hereinabove, seemingly slight changes in the chemical structure of the emulsion addenda employed in the practice of this invention have a marked

70 We claim:

1. A photographic silver halide emulsion stabilized with a compound having the formula:



65 where each R is selected from the group consisting of alkyl, trifluoromethyl and aryl.

2. A photographic silver halide emulsion stabilized with about .001 to about 10 grams per mole of silver halide of a compound having the formula:



75 where each R is selected from the group consisting of alkyl, trifluoromethyl and aryl.

3. A photographic silver halide emulsion stabilized with about .1 to about 1 gram per mole of silver halide of a compound having the formula:



where each R is selected from the group consisting of alkyl, trifluoromethyl and aryl.

4. A photographic silver halide emulsion stabilized with a compound having the formula:



where each R is an alkyl radical containing up to 20 carbon atoms.

5. A photographic silver halide emulsion stabilized with a compound having the formula:



where each R is an alkyl radical containing 1-10 carbon atoms.

6. A photographic silver halide emulsion stabilized with about .1 to about 1 gram per mole of silver halide of a compound having the formula:



where each R is an alkyl group containing 1-10 carbon atoms.

7. A photographic silver halide emulsion stabilized with a compound having the formula:



where each R is an aryl radical containing up to 20 carbon atoms.

8. A photographic silver halide emulsion stabilized with about .001 to about 10 grams per mole of silver halide of bis(p-trifluoroacetamidophenyl) disulfide.

9. A photographic silver halide emulsion stabilized with about .001 to about 10 grams per mole of silver halide of bis(p-acetamidophenyl) disulfide.

10. A sulfur and gold sensitized negative, high speed gelatino silver halide emulsion stabilized with about .001 to about 10 grams per mole of silver halide of a compound having the formula:



where each R is an alkyl radical containing up to 20 carbon atoms.

11. A sulfur and gold sensitized negative, high speed gelatino silver halide emulsion stabilized with about .001 to about 10 grams per mole of silver halide of bis(p-acetamidophenyl) disulfide.

12. A high speed gelatino silver bromoiodide emulsion stabilized with about .25 gram per mole of silver halide of bis(p-acetamidophenyl) disulfide.

13. A high speed orthochromatically sensitized gelatino silver bromoiodide emulsion stabilized with about .25 gram per mole of silver halide of bis(p-acetamidophenyl) disulfide.

14. A sulfur and gold sensitized negative, high speed gelatino silver bromoiodide emulsion which is stabilized with about .09 gram per mole of silver halide of bis(p-acetamidophenyl) disulfide.

#### References Cited

##### UNITED STATES PATENTS

35 1,962,133 6/1934 Brooker et al. ----- 96—109  
2,756,145 7/1956 Ballard ----- 96—109

NORMAN G. TORCHIN, Primary Examiner.

40 R. E. FICHTER, Assistant Examiner.